

# UNITED STATES PATENT OFFICE.

WILLIAM S. WALKER AND JARVIS L. MILLER, OF COLORADO SPRINGS,  
COLORADO.

## WATER-PROOF ROOF-PAINT.

SPECIFICATION forming part of Letters Patent No. 364,065, dated May 31, 1887.

Application filed March 16, 1887. Serial No. 231,166. (No specimens.)

*To all whom it may concern:*

Be it known that we, WILLIAM S. WALKER and JARVIS L. MILLER, citizens of the United States, and residents of Colorado Springs, in the county of El Paso and State of Colorado, have invented certain new and useful Improvements in Water-Proof Roof-Paints; and we do declare the following to be a full, clear, and exact description of the invention, such as will enable others skilled in the art to which it appertains to make and use the same.

Our invention relates to a composition of matter which we design for a roofing-paint and as a cement for stopping leaks; and it consists of the following ingredients, combined in the proportions stated, viz: coal-tar, five gallons; asphaltum varnish, one quart; Japan varnish, one quart; crude carbolic acid, one pint.

The above ingredients are stirred briskly for

about twenty minutes, and then thinned to the desired consistency with equal parts of naphtha and lime-water and applied to the roof with a large brush.

What we claim, and desire to secure by Letters Patent, is—

The herein-described composition of matter to be used for painting and cementing roofs, consisting of coal-tar, asphaltum varnish, Japan varnish, crude carbolic acid, naphtha, and lime-water, in the proportions specified.

In testimony whereof we affix our signatures in presence of two witnesses.

WILLIAM S. WALKER.  
JARVIS L. MILLER.

Witnesses:

J. W. WORK,  
F. B. WELLS.